

Feb. 27, 1934.

M. O. SCHUR

1,948,944

PROCESS OF PRODUCING NITROCELLULOSE

Filed July 17, 1930



Inventor  
Milton O. Schur  
by Wright Brown Quincy May  
Attys

## UNITED STATES PATENT OFFICE

1,948,944

## PROCESS OF PRODUCING NITROCELLULOSE

Milton O. Schur, Berlin, N. H., assignor to Brown Company, Berlin, N. H., a corporation of Maine

Application July 17, 1930. Serial No. 468,529

10 Claims. (Cl. 260—145)

This invention relates to a process of producing nitrocelluloses, and, while not restricted thereto, it is concerned with a process in which a compact or dense form of cellulose is used as a raw material.

In the nitrocellulose industry, it has heretofore been the general custom to use cellulose in bulky form as a raw material, for instance as linters, shredded paper, pulp, etc. Such raw material requires a large amount of nitrating acid in order to be properly nitrated. In fact, the ratio of nitrating acid to dry cellulose required is usually a minimum of about fifty to one. This means that a large excess of nitrating acid is constantly tied up in the process, and further that this acid must be handled along with the cellulose as a bulky mass after nitration has been completed, that is, up to the point where the excess acid is separated out as by centrifugation. The large excess of acid present during the nitrating operation, however, ensures a nitrating acid of practically fixed composition, since the generation of water during nitration and the consumption of nitric acid effects but a negligible weakening of the acid.

In accordance with the present invention, I preferably use a compact or dense form of cellulose as a raw material for making nitrocelluloses. More particularly, I prefer to use a nitration grade of wood pulp in the form of comparatively thick sheets or boards known in the trade as "drier sheets." These sheets are supplied by pulp manufacturers, who find it economical practice to run off their processed pulps on pulp driers which may be built as large units capable of handling 100 or more tons of pulp per day. Various types of wood pulp are sold in such form,—for instance, the sulphite pulp used by viscose-rayon manufacturers. For nitration purposes, however, the wood pulp should preferably be a pure white, refined product of high alpha cellulose content, low soda solubility, and other characteristics specified by nitrocellulose converters. The sheets, which may be of a thickness of, say, 0.020 to 0.050 inches, are compact or dense, as compared with cotton linters, because of the interfelted relation of the fibers. When such sheets are nitrated by steeping in a bath of nitrating acid, a much lower ratio of nitrating acid to dry fiber is necessary to ensure complete submergence of the sheets than that necessary in the case of a bulky material such as cotton linters, but if this ratio is too low, the acid is so weakened as nitration proceeds that it will fail to nitrate properly. In accordance with the present inven-

tion, a comparatively low acid to fiber ratio is employed in the nitrating vat, for instance, less than about forty to one, but as nitration proceeds, acid of the desired composition is progressively fed into the vat while the acid is being progressively withdrawn from the vat, preferably at a point remote from the point of feeding, for fortification and reuse, so that there is a constant circulation of acid of the desired composition in the vat to ensure proper nitration. Whereas circulation of acid through a bulky mass is not entirely practicable, with dense sheets it is easy to afford such circulation while a bath of comparatively low acid to fiber ratio is being maintained in the nitrating vat. Such a procedure is advantageous, in that it permits a high nitrocellulose production with comparatively little nitrating acid being tied up in the process, as I may provide a master pool or reservoir of excess acid of the proper composition for a large number of nitrating vats or units. Acid may be constantly supplied in regulated amount from the master pool to each of the nitrating units while acid is being constantly withdrawn from the nitrating units, fortified, and returned to the reservoir. Such a procedure is further advantageous, in that the nitrating units may be of small size because of the compactness of the cellulose and the comparatively small volume of acid present therein during the nitrating operation.

A further advantage of my process is that the temperature of all the baths of acid may be easily maintained substantially constant throughout the nitrating acid, since it is necessary to control only the temperature of the master pool of acid for this purpose. As is well known to those skilled in the art, the quality or grade of nitrocellulose is affected not only by the composition of the nitrating acid, but also by the temperature maintained during the nitrating operation. By applying my invention, therefore, it is possible to regulate closely the quality of the nitrocellulose produced.

The master pool may be of sufficient volume so that it is unnecessary to fortify the acid being withdrawn from the nitrating units and returned to the pool, particularly if the acid is circulated through the baths at a rate ensuring the recirculation of the total quantity of nitrating acid from the master pool through the baths a plurality of times during a nitrating operation, as in such case the acid in the baths is maintained substantially fixed in composition. It is, however, preferable to fortify the acid being withdrawn from the baths before it is returned to the master

pool, as in such case the total quantity of acid in the system may be far less than that necessary when a bulky form of cellulose such as cotton linters is employed as a raw material. In any event, however, the system is preferably operated so that the total volume of acid being used therein makes a number of circuits through the nitrating units, as such mode of operation makes possible nitration under substantially fixed conditions of both acid composition and temperature in the baths.

With these and other objects and features in view, my invention will now be described with greater particularity in conjunction with the accompanying drawing, which illustrates more or less diagrammatically and conventionally an apparatus embodying the principles of the invention.

Referring to the drawing, 1, 2 and 3 represent a series of closed nitrating vats or units in which the nitration of sheets of cellulose of the kind described may be carried out. The walls of vat 1 are shown partly broken away, to illustrate how sheets 4 may be arranged inside the vat in closely spaced, parallel relation, as by suspension from rods 5. Nitrating acid of the desired composition may be supplied to the vats in amount sufficient to submerge the sheets from a storage tank 6 shown located above the vats and in which a master pool of nitrating acid may be kept for the nitrating baths. A coil 7, through which a heating or cooling medium may be passed, is shown within the tank 6, so that the master pool may be maintained at the desired temperature. The acid may be allowed to gravitate from the tank 6 through a pipe 8 into a manifold 9 which leads the acid through a series of valved connections 11, each of which enters into a vat through its end 10, preferably near its bottom. Communicating by means of valved connections 25 with the vats through their other ends 12, preferably near their tops, is a manifold 13, which is connected by a pipe 14 to a pump 15 by which the acid may be withdrawn from the vat and fed through a pipe 16 into a chamber 17, shown above the vats. Preferably also a series of valved bottom connections 26 are provided between the vats and the manifold 13, which will permit removing all the acid from the vats by the pump 15 when the nitrating operation has been completed. By feeding acid into each vat at one end near its bottom and withdrawing it at the other end near its top, a positive flow and diffusion of acid of the desired composition is ensured through each vat and the accumulation of weakened acid at any point in the bath is avoided.

The acid fed into the chamber 17 may be fortified or strengthened to the desired composition by delivering fortifying acid in regulatable quantities thereinto as from a doser 18 located above the chamber and supplied with acid by gravity from a storage tank 19 located thereabove, in which a supply of the fortifying acid is kept. A stirrer 20 is preferably provided in the chamber 17 to effect a uniform mixture of the acids. The fortified acid may gravitate from the chamber 17 through a pipe 21, valved as at 22, into a pump 23 which discharges into the top of the tank 7 through a pipe 24.

When nitration is going on, there is a constant circulation of acid in the system from the storage tank 7 through the nitrating vats, through the mixing chamber 17, back to the storage tank 7, the acid withdrawn from the vats being dosed in the chamber 17 with the appropriate amount

of fortifying acid to restore it to the desired condition. This circulation is preferably carried on at such a rate that the total volume of acid in the system completes a plurality of circuits during a single nitrating operation, so as to ensure practically constant nitrating conditions in each nitrating vat. In operating the apparatus described it is unnecessary to start all the vats at once. In fact, it may be desirable that charge of cellulose at various stages of reaction are in process in the vats at any one time, as this would not only tend to keep the composition of the acid circulation through the system more nearly uniform, but would also tie in better with the operations of charging, washing, drowning, stabilizing, etc.

The principles of the present invention may be applied when the sheets are cut into small pieces, for by providing strainers or screens at the points of communication of the manifolds 9 and 13 with the vats, the pieces may be kept in the vats, but in such case stirrers are preferably also provided in the vats, so as to offset the tendency for the pieces to accumulate or pack at the regions where acid is being withdrawn. Ordinarily, however, it is preferable to use sheets of comparatively large size suspended from rods or held in suitable clamps or frames. They are maintained entirely submerged in the nitrating acid, so that the nitrating acid may contact uniformly with all the surface presented and effect a uniform nitration. Such large sheets may be handled readily as such through the after-nitration treatments, and constitute an economical and convenient form in which to store, pack, and ship the finished product.

I claim:

1. A process which comprises steeping compact sheets of cellulose as a stationary batch in a bath of nitrating acid of the desired composition, and progressively feeding acid of said desired composition into the bath while progressively withdrawing acid from the bath as nitration proceeds.

2. A process which comprises steeping compact sheets of cellulose as a stationary batch in a bath of nitrating acid of the desired composition, and as nitration proceeds progressively introducing acid of said desired composition into the bath while progressively withdrawing acid from the bath at a point remote from the point of introduction of acid.

3. A process which comprises steeping compact sheets of cellulose as a stationary batch in a bath of nitrating acid of the desired composition, progressively feeding acid of said desired composition into the bath while progressively withdrawing acid from the bath as nitration proceeds, fortifying said withdrawn acid to said desired composition, and using it as the acid for feeding into the bath.

4. A process which comprises steeping compact sheets of cellulose as a stationary batch in a bath of nitrating acid of the desired composition, maintaining an independent pool of acid of said composition, progressively feeding acid from said pool into said bath while progressively withdrawing acid from said bath, fortifying said withdrawn acid to the desired composition, and delivering said fortified acid into said pool.

5. A process which comprises steeping compact sheets of cellulose as stationary batches in a plurality of baths of nitrating acid of the desired composition, maintaining a master pool of acid of said desired composition for said baths, progressively feeding acid from said pool into said

- baths while progressively withdrawing acid from said baths, fortifying said withdrawn acid to the desired composition, and delivering said fortified acid into said pool.
- 5 6. A process of nitrating compact sheets of cellulose as stationary batches in a plurality of nitrating baths, which comprises maintaining a master pool of nitrating acid in which said sheets are submersed in circulating communication with each of the baths, and while nitration is in progress causing progressive circulation of the acid from the master pool through the baths at a rate ensuring the recirculation of the total quantity of acid a plurality of times.
- 10 7. A process which comprises nitrating compact sheets of cellulose as a stationary batch in which the ratio of nitrating acid to such cellulose in the reaction vessel is less than about 40 to 1 throughout the nitrating reaction and in which the nitrating acid is fortified during the course of the reaction on such cellulose.
- 15 8. A process which comprises nitrating compact
- 10 sheets of cellulose as a stationary batch in which the ratio of nitrating acid to such cellulose in the reaction is initially less than 40 to 1, and maintaining the composition of the nitrating acid and its ratio to the cellulose substantially constant until nitration has been completed.
- 15 9. A process which comprises nitrating compact sheets of cellulose as a stationary batch in a bath of nitrating acid, and uniformly and progressively fortifying the nitrating acid in said bath to maintain its composition substantially constant throughout the nitrating operation.
- 20 10. A process which comprises nitrating compact sheet of cellulose as a stationary batch in which the ratio of nitrating acid to cellulose in the reaction is initially less than 40 to 1, and uniformly and progressively fortifying the nitrating acid in said batch with fresh reagents to maintain the composition of the nitrating acid and its ratio to the cellulose substantially constant until nitration has been completed.

MILTON O. SCHUR.

|    |     |
|----|-----|
| 25 | 100 |
| 30 | 105 |
| 35 | 110 |
| 40 | 118 |
| 45 | 120 |
| 50 | 125 |
| 55 | 130 |
| 60 | 135 |
| 65 | 140 |
| 70 | 145 |
| 75 | 150 |